

May 12, 1931.

A. JONES

1,805,144

MANUFACTURE OF PRINTED FLOOR COVERINGS

Filed Aug. 13, 1926



*Fig. 1.*

INVENTOR  
*Alfred Jones*  
by his attorney  
*Hyatt, Stetson & Banks*

## UNITED STATES PATENT OFFICE

ALFRED JONES, OF LANCASTER, PENNSYLVANIA, ASSIGNOR TO ARMSTRONG CORK COMPANY, OF LANCASTER, PENNSYLVANIA, A CORPORATION OF PENNSYLVANIA

## MANUFACTURE OF PRINTED FLOOR COVERINGS

Application filed August 13, 1926. Serial No. 129,026.

This invention relates to the manufacture of printed floor coverings, such as linoleum, felt base floor coverings, and the like, the practice of the present invention comprising the subject matter of my copending application Serial No. 233,892 filed Nov. 17, 1927.

According to the present practice of printing the surface of linoleum and other floor coverings, the various colors are successively applied to the surface of the floor covering by means of vertically reciprocal printing blocks. These printing blocks have a printing surface which is formed of a plurality of very small pegs, usually of wood, each peg being separated from the adjacent ones. This is necessary in order to get a smooth distribution of the paint and allow for the escape of air when the printing block comes down on to the material and to allow air to enter under the block when the block raises from the printed surface.

Heretofore the usual slow drying oil paints have always been used in machines of this character as the coating material. Due to the fact that the paint is necessarily slow drying, a very large amount of curing space, or stove room, is necessary for taking care of the output of a single machine, as the freshly painted material must cure for several days before it can be further handled. Furthermore, any paint used on a floor covering is subjected to the action of alkalies in soaps, and these alkalies are detrimental to ordinary oil base paints.

According to the present invention it is proposed to use a nitrocellulose lacquer as a vehicle for the print paints, thus eliminating the use of linseed or other drying oils in order to produce a paint which is highly resistant to the action of alkalies and soaps commonly used for the cleaning of floor coverings.

Furthermore, nitrocellulose lacquers are quick drying, and consequently the material can be handled much more quickly after it has been printed, and the amount of storage or curing space necessary to take care of the output of a single machine is materially reduced.

There are several lacquer paints now on the market which can be applied with a brush or

with a spray, but no lacquer paint has heretofore been produced which can be used on printing machines of the type used in the decorating of floor coverings. The greatest difficulty, in connection with all of these paints up to the present time, is their tendency to set, due largely to the fact that they are quick drying, thereby choking up the printing blocks and preventing the machines from operating on a production basis.

It is proposed by the present invention to provide a method by means of which nitrocellulose lacquers commonly called lacquer paints can be practically used with present types of printing machines without choking the printing blocks, and to produce a printed floor covering wherein the paint is highly resistant to the action of alkalies. The present invention also contemplates the provision of novel apparatus by means of which the invention can be most effectively and economically practiced.

The invention may be readily understood by reference to the accompanying drawings in which:

Figure 1 is a diagrammatic vertical section taken longitudinally of a printing machine and curing stove;

Figure 2 is a perspective view showing a portion of one of the printing blocks to illustrate the peg-like structure of the printing surface.

In the drawings, 2 designates the bed of a standard type of printing machine and 3 are the vertically reciprocal printing blocks. These blocks have a sawed or peg-like printing surface 4, as clearly shown in Figure 2. By reference to Figure 2, it will be seen that the printing surface, which is of a divided nature projects beyond the general surface of the block, and it is to this portion of the block that the paint material is applied and it is this portion of the block that engages the linoleum or other floor covering to reproduce the pattern thereon. A web 5 of linoleum or other floor covering material is guided over the bed 2 below the reciprocal printing heads 3. The linoleum passes from the printing machine directly into a curing stove 6 wherein it is vertically festooned for

drying. Provision is preferably made for heating the stoves or curing rooms 6, although such means has not been shown in the drawings. Provision is made for withdrawing vapors from the stove in order to collect the solvents of the nitrocellulose lacquer as the same dries. For this purpose I have illustrated a pipe 7 leading to a suction fan 8 which may discharge into any suitable condensing apparatus, not shown, in order to effect a recovery of the vapors.

It has previously been pointed out that nitrocellulose lacquers or lacquer paints have a tendency to choke the surfaces 4 of the printing blocks and that this interferes with the practical operation of the machine. In order to maintain an atmosphere about the machine which precludes any substantial degree of evaporation of the low boiling point solvents, the machine is preferably placed in an enclosed room 9 which may be maintained at a temperature most conducive to the securing of satisfactory results. I have indicated cooling coils 11 in the room so that the atmosphere about the machine may be cooled to the extent desired. In practice the atmosphere will be kept at a temperature of approximately 60° F.

For the purpose of maintaining an atmosphere about the machine itself which is highly saturated with solvents, a wall 12 is preferably built around the machine to a height slightly above the highest point of travel of the printing blocks. The solvent vapors which are heavier than air, will be confined in this enclosure so that a highly saturated atmosphere will exist around the printing blocks. This will practically eliminate evaporation of the lacquer on the block, so that the block will not become choked. At the same time the enclosure will not interfere with workmen in their operation of the machine.

By maintaining a low temperature and a solvent saturated atmosphere about the machine, practical operation with nitrocellulose lacquers can be carried on.

The materials which may be used will consist of a solution of nitrocellulose in suitable solvents, together with plasticizers or softeners, gums or resins, any desired pigments or fillers to produce the right shade, and any non-solvents for nitrocellulose which are volatile and which may be used either as cheap thinners or as solvents for the resins.

The nitrocellulose will be the soluble form of the product of nitration of cellulose, of which cotton is the usual source. It is preferably of a type which forms solutions of low viscosity.

The solvents may be any of the materials that dissolve or disperse nitrocellulose. These may be alcohols, ethers, esters, ketones, aldehydes, or any combinations of these substances, and may fall into any or all of the

classes commonly known as low, medium, or high boiling solvents.

Among the latter known substances now in use are methyl, ethyl, butyl, amyl, and the higher alcohols, which may be monohydric, di-hydric or higher; acetone, ethyl methyl ketone, or any of the higher ketones including the ketone alcohols, such as diacetone alcohol; the acetates, butyrate, propionate, lactates, phthalates, carbonates, or other esters of methyl, ethyl, butyl, amyl, or other alcohols. Certain other compounds such as some aldehydes, so-called oxides, and camphor might also be used, but it is to be understood that the invention is not limited to any of these specific solvents mentioned.

The plasticizers or softeners may be any of the common vegetable oils such as rape, castor, linseed, china wood, perilla, or other non-drying, semi-drying, or drying fatty oils; the phosphates of organic radicals such as the di- or triphenyl or cresyl phosphates; the stearates, tartrates, phthalates, lactates or other non-volatile softening materials soluble in the nitrocellulose solvents and being preferably, but not necessarily, solvents for nitrocellulose. Resins may or may not be used, depending on the type of paint or surface desired. Examples of such materials which can be used are rosin, ester gum, shellac, dammar, gilsonite, manila or pontianak, any of the copals, or various synthetic resins.

The pigments which are used may be any of the pigments now commonly used in paints or other decorative coatings, such as lithopone, zinc oxide, titanium oxide, oxides of iron, Prussian or ultramarine blues, chrome or iron yellows and greens, any of the forms of carbon black, and any of the lake colors.

Non-solvents may or may not be used as diluents or as solvents for the resins. Some of these non-solvents are hydrocarbons of the aliphatic or aromatic series, or certain alcohols which alone have little or no solvent action on nitrocellulose.

Where the oils mentioned are used as the plasticizers, the preferred method is to grind the pigment in all or part of this oil. The paste which results is then mixed in the previously prepared nitrocellulose solution, which may also contain the remaining part of the plasticizer, if any, and the resin. The paint is then thinned for use with any of the above solvents or non-solvents, or combinations thereof.

Another procedure which has been found satisfactory in all cases, but especially so where solid plasticizers are used, consists of mixing all the ingredients in a closed container, such as a ball or pebble mill. This method may be varied somewhat by dissolving the nitrocellulose and resin separately in suitable solvents, the two solutions then being mixed with plasticizers and the entire

mixture being ground with the pigment as above suggested. The thinning to printing consistency is then done as before described.

From the foregoing it will be seen that 5 there is a very wide choice of materials possible and the number of variations in composition is almost infinite. It has been found, however, that where the composition is to be used on printing blocks in a normal 10 atmosphere, that it is necessary to use a large proportion of the high boiling point solvents. By chilling the atmosphere around the printing machine, as may be done where the printing machine is enclosed, as herein- 15 before described, or by saturating the atmosphere surrounding the printing operation with vapors of the solvent, low boiling point solvents may be used, and these are considerably cheaper.

20 A few examples of compositions which have been successfully used for block printing of floor coverings are as follows:

*Formula #1*

|                                                                                                                                                                     | Parts |
|---------------------------------------------------------------------------------------------------------------------------------------------------------------------|-------|
| Nitrocellulose solution (20 oz. nitrocel-<br>lulose to gallon of ethyl acetate)                                                                                     | 100   |
| Castor oil                                                                                                                                                          | 50    |
| Pigment                                                                                                                                                             | 50    |
| 30 Grind pigment separately in a portion of<br>the castor oil, mix all ingredients and thin to<br>desired consistency with equal parts butyl<br>acetate and toluol. |       |

*Formula #2*

|                                    | Parts |
|------------------------------------|-------|
| Nitrocellulose solution (as in #1) | 125   |
| Ester gum                          | 15    |
| Butyl phthalate                    | 30    |
| Pigment                            | 60    |

40 The ester gum is dissolved in the butyl phthalate and the pigment ground in this solution; all ingredients are then mixed and the whole is thinned to proper consistency 45 with diacetone alcohol and toluol.

*Formula #3*

|                                    | Parts |
|------------------------------------|-------|
| Nitrocellulose solution (as in #1) | 125   |
| Tri-phenyl phosphate               | 30    |
| 50 Manila gum                      | 15    |
| Pigment                            | 60    |

55 The Manila gum is dissolved separately in a small quantity of ethyl alcohol and all ingredients are ground in a ball mill finally thinned with ethyl lactate, ethyl alcohol, and toluol.

*Formula #4*

|                                            | Parts |
|--------------------------------------------|-------|
| 60 Lacquer (20 oz. ethyl acetate solution) | 120   |
| Butyl phthalate                            | 20    |
| Ester gum                                  | 30    |
| Pigment                                    | 60    |

65 About five parts of the ester gum are dissolved in the butyl phthalate and the pig-

ment ground in this solution. The remainder of the gum is dissolved in a portion of the diacetone alcohol which is used for thinning. The paste of pigment, butyl phthalate, gum solution and diacetone gum solution are all 70 thoroughly mixed and then thinned to printing consistency.

After any of the above compositions have been made they are then applied to the printing blocks, which may be either hand manipulated blocks, or be machine operated blocks, as hereinbefore described and applied to suitably prepared linoleum, felt base, or other hard surfaced floor covering material. As 75 many different colors may be applied as are desired, and the paints may be applied either to a rug design or to a continuous design. The operation of printing is substantially the same as that carried out with the present oil paints except that the machine is preferably 80 enclosed in order to reduce evaporation of the low boiling solvents and thereby prevent a clogging of the printing blocks. By reference to Figure 2, it will be readily seen that the blocks might easily become clogged if 85 care is not taken to prevent evaporation of the solvents.

The pigment may be applied to the printing blocks in any of the usual ways, the drawing showing reciprocating pots of the usual 90 type for this purpose. The pots are designated 10.

The drying of the pattern after it has been 95 printed is done either at normal or elevated temperatures, as hereinbefore described. The 100 solvents may or may not be recovered, although in the present application I have illustrated means for withdrawing the vapors from the drying chamber.

The evaporation of the solvent and the 105 consequent setting of the nitrocellulose, both on the goods and on the printing blocks is retarded considerably by maintaining a reduced temperature around the printing apparatus, as well as by operating the machine 110 in a solvent laden atmosphere.

I am aware of the fact that nitrocellulose 115 lacquers and paints are at the present time well known, and that it has been proposed to apply such lacquers and paints to floor coverings by means of sprays or brushes, but heretofore, so far as I am aware, no process has been developed by means of which a lacquer can be applied to a floor covering in a commercially practical manner by means of 120 a block printing process.

If desired, a top coating of clear lacquer could be applied over the lacquer paint to afford protection thereto.

An important advantage in the use of a 125 lacquer paint is the fact that it dries quickly, eliminating some of the present curing time, so that less space in the curing chambers or stoves is required. A further important advantage is that the printed colored 130

pattern is more resistant to alkaline soaps and cleansers than is an oil paint.

While I have described and shown certain methods and apparatus for carrying out the invention, it will be understood that the invention is not restricted to the particular methods and apparatus disclosed, these being merely illustrative of the spirit of my invention, and various changes and modifications may be made therein within the scope 10 and contemplation of my broader claims.

I claim:

1. The method of applying lacquer paint to a floor covering which consists in applying 15 the paint first to a printing block, and pressing the printing block against the floor covering while maintaining an atmosphere about the printing block which precludes any substantial evaporation of the lacquer solvents 20 on the printing block.

2. The method of applying pigment bearing nitrocellulose lacquer containing low boiling point solvents to floor coverings which consists in applying the lacquer to printing 25 blocks, pressing the printing blocks against the floor covering, and maintaining an atmosphere about the printing blocks saturated with the low boiling point solvents whereby 30 any appreciable evaporation of the solvents from the lacquer applied to the printing blocks is precluded.

3. The method of applying lacquer paint to floor coverings in a block printing machine which consists in operating the machine in 35 an atmosphere which precludes evaporation of the solvents of the lacquer paint during the printing process.

4. The method of applying lacquer paints to a floor covering by means of a block printing 40 machine which consists in maintaining an atmosphere around the machine which is saturated with solvents contained in the lacquer paint whereby any choking of the printing blocks with the paint is avoided.

45 5. The method of printing a multi-colored pattern on a floor covering material with a lacquer paint which consists in passing the floor covering material under a series of printing blocks arranged to apply different colored lacquer paints thereto while maintaining the material and the printing blocks in an atmosphere which substantially precludes evaporation of the solvents from the lacquer, whereby the printing blocks are prevented from becoming choked with the lacquer paint, and subsequently exposing the 50 printed material to an atmosphere conducive to the evaporation of the solvents.

6. The method of surfacing floor covering 60 materials which consists in applying lacquer paint to the surface of the material by means of printing blocks under conditions which preclude any substantial evaporation of the solvents from the lacquer paint, and then 65 curing the paint in an atmosphere con-

ducive to the rapid evaporation of the solvents therefrom.

7. The method of surfacing floor covering materials with lacquer paint which consists in applying the paint to the material in a block printing machine, maintaining an atmosphere about the machine saturated with solvents from the lacquer paint, then introducing the product to a curing chamber, and withdrawing the vapors of the solvents from the curing chamber to facilitate the rapid removal thereof. 70 75

8. Apparatus for applying lacquer paint to floor coverings comprising a block printing machine and an enclosing casing therefor by means of which an atmosphere may be maintained about the machine which precludes the evaporation of the solvents from the lacquer paint. 80

9. Apparatus for applying lacquer paint to the surface of floor coverings comprising a block printing machine, an enclosing housing therefor in which a saturated atmosphere can be maintained, a curing chamber to which the printing machine delivers, and means for withdrawing vapors from the curing chamber. 85 90

10. The method of applying lacquer paints to floor coverings which consists in applying the paint to a printing surface and then pressing the surface against the floor covering while maintaining an atmosphere of reduced temperature saturated with solvents from the lacquer about the printing surface. 95

11. The method of applying lacquer paints to a floor covering by means of a block printing machine which consists in maintaining an atmosphere around the machine which is saturated with solvents contained in the lacquer paint whereby any choking of the printing blocks with the paint is avoided, and while maintaining such atmosphere at a reduced temperature. 100 105

12. Apparatus for applying lacquer paint to floor coverings comprising a block printing machine and an enclosing casing therefor by means of which an atmosphere may be maintained about the machine which precludes the evaporation of the solvents from the lacquer paint, and means for cooling the atmosphere about the machine. 110 115

13. Apparatus for applying lacquer paint to floor coverings including a block printing machine, an enclosure around the sides of the machine open at its top, a room in which the machine is located, and means for cooling the atmosphere in the room. 120

14. The method of applying lacquer paints to a floor covering which comprises applying the paint to the material in a block printing machine, the paint having a solvent, trapping the evaporated solvent, and maintaining it in the atmosphere surrounding the machine. 125

15. The method of applying lacquer paints 130

to a floor covering which comprises applying the paint to the material in a block printing machine, the paint having a solvent, trapping the evaporated solvent, maintaining it in the atmosphere surrounding the machine, and controlling the temperature of the solvent-laden atmosphere.

16 16. The method of applying lacquer paints to a floor covering which comprises applying the paint to the material in a block printing machine, the paint having a solvent, trapping the evaporated solvent, maintaining it in the atmosphere surrounding the machine, and cooling the solvent-laden atmosphere.

15 17. The method of applying lacquer paints to a floor covering which comprises supplying paint in a solvent to a block printing machine for the application thereof to the material, and blocking escape of evaporated 20 solvent around the sides of the machine to a height above that of the printing surfaces.

25 18. Apparatus for applying lacquer paint to floor coverings comprising a block printing machine and an enclosure therefor, said enclosure being arranged so that the material to be printed travels therethrough.

In testimony whereof I have hereunto set my hand.

ALFRED JONES.

30

35

40

45

50

55

60

65